

## UNITED STATES PATENT OFFICE

TREADWAY B. MUNROE AND ELBERT C. LATHROP, OF CHICAGO, ILLINOIS, ASSIGNEES  
TO THE CELOTEX COMPANY, OF CHICAGO, ILLINOIS, A CORPORATION OF DELAWARE

## TREATMENT OF FIBER PRODUCTS

No Drawing.

Application filed December 27, 1930. Serial No. 505,203.

In the past, various fibrous materials, for example the various paper making fibers, board fiber, and the like, have been sized and various treatments have been employed to 5 make the products produced therefrom fungi-proof and repellent to or toxic to insects. While some of the heretofore proposed treatments have produced satisfactory sizing and some have provided the desired resistance to 10 fungi and toxicity to insects, there has been, so far as is known, no treatment developed which as a single treatment provides integrally all the desired properties of products produced from fibers.

15 Some of the proposed sizing treatments have been detrimental to the treatments designed to produce fungi and insect proofing and some fungi and insect proofing treatments have been detrimental to sizing treatments, and in fact so far as can be determined the problem of providing a satisfactory fiber treatment affording the several properties of water proofing, fungicidal protection and toxicity to insects has seemed 20 utterly impossible of solution.

In its broadest application this invention comprehends the use of a water solution of arsenic, in any form, in which while having the pulped material in suspension therein, 25 a precipitating agent is added to precipitate a relatively insoluble simple or complex arsenical.

It is a particular object of this invention to provide a treatment of fiber whereby there 35 is provided an integral water proofing which at the same time provides the desired resistance to fungi and toxicity to insects which treatment may comprise a single step of application or which may be accomplished by 40 a plurality of succeeding steps of treatment. The invention from the aspect just stated involves primarily the introduction of arsenic into a mass of fibers wherein the arsenic is caused to adhere to the fibers thereof by the 45 addition of iron salts, primarily ferric chloride or ferrous sulphate, and which with the further inclusion of a size, as rosin, resin, paraffin, wax, bituminous material or the like, affords the desired water proofing or 50 sizing of the fiber.

An additional object of the invention is to provide a treatment as above described which will afford a means of maintaining a uniform color of the products produced from the fiber which has been treated therewith.

Particularly in the manufacture of insulating boards, due to the fact that they are largely manufactured of raw materials seasonably obtained from vegetative sources, it is common for the color to vary in accordance 55 with the length of time that the basic fibrous material has been in storage. As a means of maintaining a uniform coloration of the final product, it is an object of this invention to provide a treatment by means of which there 60 is afforded the desired sizing, fungi proof-ness and insect toxicity which in addition provides a treatment whereby a uniform color or may be maintained in the finished product.

Other and further objects of the invention are to provide a fiber treatment as above described which is applied integrally to the fiber prior to its formation into the finished product, whereby it may be uniformly and 65 thoroughly distributed throughout the final product, and in addition, to provide a treatment which is relatively cheap, is applied at small cost, is easily applied, and wherein the losses of the various chemicals used may be 70 maintained at a minimum. Still other and further objects of the invention will be apparent on reading the following detailed 75 specifications of the invention, wherein there is particularly set forth a preferred treatment.

Paper, fiber boards, and the like, are made from more or less finely divided fibrous materials, principally from cotton, various woods, and other vegetative growth, such as 80 corn stalks, sugar cane bagasse, straws, and the like. In general the raw material is prepared for use in the manufacture of the various finished products by means of some form of digestion and mechanical refining 85 which serves to more or less soften the raw materials and subdivide them into their fiber elements or into relatively small fiber bundles.

The digested and refined fibrous material 100

is formed into paper and board products and the like by some form of felting from a diluted water suspension wherein ordinarily the fiber content of the suspension is, at the time 5 of felting, in the neighborhood of  $\frac{1}{2}\%$  and which is seldom if ever above 5% in any part of the system preceding the felting operation.

The treatment of the fiber material according to this invention takes place at any desired point between that of the subdivision 10 of the fibrous material into its fibers, or into small fiber bundles, and is preferably applied to the fiber while in the condition ordinarily referred to as half stock, at which time the 15 consistency of the fiber suspension is ordinarily between about 1 to 2 per cent.

It has been discovered that ferric chloride when added to a water suspension of fiber in the presence of hydroxyl ions probably does 20 not exist as such but quickly changes to ferric hydroxide which is adsorbed by the fiber, and that the fiber carrying the adsorbed ferric hydroxide readily absorbs arsenic which may be conveniently added to the suspension 25 as arsenious acid, and that the addition of ferric chloride and arsenious acid to a fiber suspension to which there has been previously added a sizing emulsion, will cause 30 coagulation or precipitation of the substance thereof on the fiber in addition to the adsorption as previously described.

Whereas the action just described covered only ferric chloride, it is to be noted that other iron salts or combinations thereof may 35 be substituted. An example of an alternative iron salt is ferrous chloride, or in fact the initial materials may comprise any iron salt or salts which as used are hydrolyzed to the form of a hydrated oxide of iron.

40 In applying this process to render fibrous materials toxic and water resistant, about 2% arsenic is added, conveniently as arsenious acid dissolved in caustic soda or sodium carbonate, but it is to be understood that the invention does not necessarily comprehend the 45 addition of arsenious acid only as such. Many ordinary forms of arsenic, as for example, sodium arsenite when in water solution, hydrolyze to form ortho-arsenious acid 50  $H_3AsO_3$ ; therefore throughout the specification the term "arsenious acid" is used to designate a water solution of arsenic in which the arsenic trioxide  $As_2O_3$  radical in a water soluble compound is generally the active constituent for the purpose of this invention. The invention, though, is not to be understood to be limited only to the use of water soluble arsenic compounds, as relatively insoluble arsenic compounds may be incorporated 55 by the use of a suspension thereof, or for example sodium arsenite may be used which in a water solution hydrolyzes to form arsenic acid  $H_3AsO_5$ . Other metalloids of the arsenic family, though generally less toxic, act in a manner similar to arsenic and of

course may be utilized if sufficiently toxic for the desired specific use.

The arsenious acid, as for example in the form of sodium arsenite, is preferably added to the water suspension of fiber first, and then, depending on the degree of sizing desired, there is added about 1% more or less of a suspension of a sizing agent, as for example rosin size which is the ordinary paper sizing rosin emulsion usually formed by heating and agitating the rosin with an alkali. The amount of rosin emulsion is expressed in per cent of solids in the emulsion or suspension form in which it is added. For the best and uniform results it is desirable and advisable that the arsenious acid and rosin emulsion added to the fiber suspension be fairly well mixed therewith in order that a uniform treatment may be obtained.

In using the term "sizing agent" above, it is contemplated that any of the water repellent sizing agents which are used or are usable in sizing paper and board fibers may be used, that is, rosin, resins, asphalts, waxes, paraffines, fatty acids, and the like, which sizing materials are mentioned only as illustrative and not as all-inclusive.

After the rosin emulsion and arsenious acid have been thoroughly mixed through the fluid suspension of fiber there is added approximately 2% of iron salts which in solution will form a hydrated oxide of iron, as for example ferric chloride based on the dry weight of fiber, which solution may comprise a combination of salts such as both ferric chloride and ferric sulphate, in which event this solution should be added in an amount sufficient to form the amount of hydrated oxide of iron necessary for coagulation and precipitation of the arsenic and rosin.

Upon addition of the size precipitant and coagulant to the fiber containing the arsenic and rosin, there is an action which is probably a combination of chemical and physical phenomenon whereby the arsenic and rosin are deposited on the fiber as precipitates or are adhered by absorption, or are probably more or less both deposited on and adhered to the fiber. It may be that when the ferric chloride is added the stock is outside the range of acidity or alkalinity within which the sizing, will be deposited most satisfactorily on the fibers, which range is approximately between the pH of 4.0 and 8.0, in which case an adjustment may be made with sodium hydroxide or other alkali to bring the pH within the most satisfactory range, which for the purpose of the invention, when using ferric chloride and sodium arsenite, is apparently a pH of between 4.5 and 5.5. The action in this method of sizing and providing fungi and insect proofing of the board is apparently due to the fact that the ferric chloride reacts to form ferric hydroxide, a hydrated oxide of iron, or basic ferric salts

under conditions of and within the pH range of the treatment. The ferric hydroxide apparently acts on the rosin emulsion in the same general manner as does alum with the result that apparently a resinate of iron is deposited on the fiber in the place of the alum resinate ordinarily present in the usual rosin sizing. The ferric hydroxide or other basic ferric salts formed on the addition of ferric chloride to the fiber suspension not only acts to precipitate the rosin from the rosin emulsion but it at the same time is apparently adsorbed by the fiber, and in turn absorbs the arsenic.

It is apparently of considerable advantage to form the colloidal precipitate of ferric hydroxide in place in the fiber suspension since it is quite evident that freshly formed ferric hydroxide is much more active in absorbing arsenic than is ferric hydroxide which has been previously made and allowed to stand, and it is for this reason that the iron salt is preferably employed in the form of a soluble ferric salt.

The action of the freshly formed ferric hydroxide or basic ferric salts formed upon addition of ferric chloride to the water suspension of fiber appears to consist in simultaneous and separate actions, that is, the freshly formed ferric hydroxide apparently absorbs arsenious acid to form a complex colloid in turn adsorbed by the fiber, or possibly the action may be the other way, that is, the iron salt may be adsorbed by the fiber to in turn absorb the arsenious acid. It appears that at the same time that the physical phenomenon just mentioned takes places that there is a chemical reaction which occurs, whereby the rosin of the rosin sizing emulsion is coagulated and precipitated on the fibers. The two actions just described as possible explanations of this process appear to be carried out substantially simultaneously and independently, that is, the addition of sufficient ferric chloride to absorb the arsenic is sufficient to cause the coagulation and precipitation of the rosin size from the rosin emulsion which has been added, otherwise additional ferric chloride is unnecessary over that used for providing only insect and fungi proofing.

It has been discovered that the amount of ferric chloride added may be increased to a number of times the minimum necessary without affecting the before described physical and chemical reactions, excepting possibly to increase the retention of arsenic, but additional ferric chloride will impart a brown color to the fiber, the intensity of which of course depends upon the amount of added ferric chloride. By varying the amount of ferric chloride, it is possible to control the shade of color imparted to the finished fiber products made from the fiber which has been treated in accordance with this invention.

Should the color imparted by the necessary amount of ferric chloride, which is ordinarily of necessity for the conservation of arsenic used somewhat in excess of the minimum, give too dark a shade of color to the fiber, a small amount of alum may be used to assist in the coagulation and precipitation of the size whereby a final product of lighter shade may be obtained. The entire precipitation may be brought about by the use of alum alone or by other appropriate precipitating agent, but of course in such case the coloring effect of the iron salt will not be had.

The general proportions heretofore given, that is, the addition of approximately 1½% arsenic, 1% of size and 2—2½% ferric chloride, will produce a board, or product, which is water, insect and fungi proofed, but with the proportions given there is some loss of arsenic that has not been absorbed by the ferric hydroxide and thereby affixed to the fibers. This loss mentioned is dictated by economic reasons in balancing the amount of ferric chloride used against arsenic loss and of course this will be somewhat increased or decreased depending upon variation of the amounts of the materials used as dictated by economic consideration for economical production.

In order that this arsenic loss just mentioned may be saved, it is of course possible to operate the process as a closed system or there has been devised a serial process whereby the arsenic which would otherwise go to waste may be advantageously used. The white water or waste water resulting from the formation of products from the fluid suspension of fiber in the manner which is well known, as for instance in the manufacture of fiber insulating board, is utilized in a similar process wherein it is sufficient to only provide a fungi proofness against wood destroying organisms without including the property of insect proofness.

The white water of the first system is used as makeup water for the second system whereby a small amount of arsenic is present in the fluid suspension of the fiber. To this fluid suspension there is added 1% of rosin emulsion and about 1½% ferric chloride, with the result that the ferric chloride coagulates and precipitates the rosin size and at the same time absorbs and attaches the arsenic to the fibers, all in a manner substantially as heretofore described, except that since there is only relatively a trace of arsenic present, preferably approximately 0.05 to 0.25 per cent, the products are rendered fungi proof only, and do not have the insect proofness afforded by a larger arsenic content.

Whereas the use of ferric chloride has been particularly described, it is to be understood that if desired equivalent results may be had by the use of ferrous sulphate, which in the solution forms ferrous hydroxide, which is eventually, in the course of the usual drying

by the application of heat, oxidized to the ferric state. It is quite unlikely that any commercial ferric chloride or ferrous sulphate shall not contain some ferrous chloride or ferric sulphate respectively, so it is to be understood that the salts are designated only according to the particular salt predominating. If chlorinated copperas is used as the source of iron salts, it is most probable that there will be at least some of each ferric chloride, ferric sulphate, ferrous chloride and ferrous sulphate present.

While in this specification there have been mentioned in various places "complex colloid" and "precipitate", attention is directed to the fact that so far as the invention hereof is concerned, the words "colloid" and "precipitate" should be used in substantially an interchangeable sense; that is, the chemistry of the reactions which occur is not in all cases clear and it is very possible—and even probable—that certain actions which are referred to as precipitations actually involve colloid phenomena, whereas certain actions referred to as colloid phenomena probably involve pure precipitation, and further it is quite probable that many of the reactions involved comprise the combination of chemical precipitation and colloid phenomena.

30 There having been above described the preferred embodiment of the invention,

We claim:

1. Fiber which is water, insect and fungi proofed with a complex colloid comprising, in part, iron, arsenic and rosin.
2. Fiber products sized and rendered fungi proof and insect toxic with rosin, arsenic and ferric chloride.
3. A vegetative fiber mass having incorporated therein a colloidal complex comprising a sizing agent, ferric hydroxide and arsenious acid.
4. Vegetative fiber to which, while in dilute suspension, there has been added arsenious acid, rosin emulsion and freshly prepared hydrous iron oxide prepared in the solution by the addition thereto of a salt comprising ferric chloride.

5. A substance having the property of water proofing, of insect toxicity and of a fungicide, comprising the complex colloid resulting from the interaction of rosin size, a water soluble arsenical embodying the arsenic trioxide radical, and a compound of iron having as an element thereof ferric chloride, when in water solution and in the presence of vegetative fiber.

6. A product comprising fibers derived from vegetative sources having incorporated integrally therein a sizing, insecticide and fungicide comprising the precipitate formed in a water solution containing rosin size, arsenious acid and hydrous ferric oxide.

7. The method of water proofing and protecting fiber derived from vegetative sub-

stances from attack by insects, fungi, and the like, comprising the incorporation therein of an insoluble colloidal complex including a sizing agent, arsenious acid and hydrous oxide of iron.

8. The method of water proofing and of protecting fiber derived from vegetative sources from attack by insects, fungi, and the like, wherein arsenious acid and a sizing agent as elements of a relatively insoluble colloidal complex are incorporated in the fiber.

9. The method of water proofing and of protecting vegetative substances from attack by insects, fungi, and the like, comprising the addition, to a water suspension thereof, of an emulsion of a sizing agent, arsenious acid, and ferric chloride, the pH of the solution adjusted to between pH 4.0 and pH 8.0 with subsequent removal of the water from the substances.

10. Vegetative fiber to which while in dilute water suspension there has been added about 2% of arsenious acid, 1% of rosin size, and 2½% of ferric salts comprising principally ferric chloride.

11. Vegetative fiber to which while in dilute water suspension there has been added about 1 to 4 per cent of arsenious acid, 0.5 to 2 per cent of rosin size and 1 to 8 per cent of ferric salts comprising principally ferric chloride.

12. Vegetative fiber to which while in water solution there has been added about 0.05 to 1.0 per cent of arsenious acid, 0.5 to 2 per cent of rosin size and 1 to 8 per cent of ferric salts comprising principally ferric chloride.

13. The method of manufacture of a water and fungi proofed board comprising the formation thereof from a water suspension of vegetative fiber containing arsenious acid, a sizing agent, and hydrated oxide of iron, and wherein the arsenious acid is supplied principally as makeup water of suspension derived from a similar like process of manufacture of fiber board but wherein the initial arsenious acid content was greater.

14. The method of serial manufacture of fiber products from fiber derived from vegetative materials wherein the first product is water, insect and fungi proofed and the succeeding product is water and fungi proofed, and wherein the first product is formed from a water suspension of fiber having distributed therethrough a complex colloid formed from principally arsenious acid, a water proofing sizing agent, and a ferric salt consisting principally of ferric chloride and the succeeding product is formed from a water suspension of fiber having distributed therethrough a complex colloid formed from principally arsenious acid, rosin size, and a ferric salt consisting principally of ferric chloride; the arsenic content of the succeeding product

- lower than that of the first product and derived from the white water or waste water of the first step of product formation to the second step as makeup water therefor.
- 5 15. Fiber products sized, rendered fungi proof and insect toxic through incorporation therein of a complex chemical colloid resulting from interaction of a sizing agent, hydrous-oxide of iron and arsenic.
- 10 16. Fiber products sized and rendered fungi proof and insect toxic with rosin, arsenic, ferric chloride, and alum.
17. A vegetative fiber mass having incorporated therein a colloidal complex comprising a sizing agent, ferrichydroxide, arsenious acid, and alum.
18. The method of rendering vegetative fiber products water repellent, insect and fungi proof, wherein the water repellent properties and the insect and fungi proofing are obtained through addition, to a dilute suspension of fiber in water, of a hydrolyzable salt of a metalloid of the arsenic family, and a water repellent paper size, the metalloid and the paper size subsequently thrown down on the fiber by the addition of a salt of a metallic element the hydroxide of which is gelatinous, the pH of the suspension being properly adjusted to a value to bring about the desired precipitation of the metalloid and the gelatinous hydrate on the fiber.
19. A vegetative fiber product rendered water repellent and insect and fungi proof by the inclusion therein of a complex colloid resulting from treatment of the fiber, while in dilute suspension, with an iron salt principally consisting of ferric chloride, a water repellent size, and a salt of arsenic which in water solution hydrolyzes to form oxide ions of arsenic.
20. A vegetative fiber product rendered water repellent and insect and fungi proof by the inclusion therein of a complex colloid resulting from treatment of the fiber, while in dilute suspension, with an iron salt principally consisting of ferric sulfate, a water repellent size, and a salt of arsenic which in water solution hydrolyzes to form oxide ions of arsenic.
- 50 21. The method of rendering vegetative fiber products water repellent, insect and fungi proof, wherein the water repellent properties and the insect and fungi proofing are obtained through addition, to a dilute suspension of fiber in water, of a hydrolyzable salt of a metalloid of the arsenic family, and a water repellent paper size, the metalloid and the paper size subsequently thrown down on the fiber by the addition of a salt of a metallic element the hydroxide of which is gelatinous, and paper makers alum, the pH of the suspension being properly adjusted to a value to bring about the desired precipitation of the metalloid and the gelatinous hydrate on the fiber.
- 55 22. The method of rendering vegetative fiber products water repellent, insect and fungi proof, wherein the water repellent properties and the insect proofing are obtained through addition, to a dilute suspension of fiber in water, of a salt of arsenic and a water repellent size, the salt of arsenic and the fiber size subsequently thrown down on the fiber by the addition of a precipitant, the pH of the suspension being properly adjusted to bring about the desired precipitation of the salt of arsenic and the size on the fiber. 70
23. The method of rendering vegetative fiber products water repellent, insect and fungi proof, wherein the water repellent properties and the insect proofing are obtained through addition, to a dilute suspension of fiber in water, of a salt of arsenic and a water repellent size, the salt of arsenic and the fiber size subsequently thrown down on the fiber by the addition of alum, the pH of the suspension being properly adjusted to bring about the desired precipitation of the salt of arsenic and the size on the fiber. 80
24. A vegetative fiber product rendered water repellent and insect and fungi toxic by the inclusion therein of a chemical complex resulting from treatment of the fiber, while in dilute suspension, with alum, a repellent size, and a salt of arsenic which in water solution hydrolyzes to form oxide ions of arsenic. 90
25. A vegetative fiber product rendered water repellent and insect and fungi toxic by the inclusion therein of a chemical complex resulting from treatment of the fiber, while in dilute suspension, with a precipitant, a repellent size, and a salt of arsenic which in water solution hydrolyzes to form oxide ions of arsenic. 95
26. A vegetative fiber product rendered water repellent and insect and fungi toxic by the inclusion therein of a chemical complex resulting from treatment of the fiber, while in dilute suspension, with alum, a repellent size, and a salt of a metalloid of the arsenic family which in water solution hydrolyzes to form oxide ions of the metalloid. 100
27. The method of rendering fibrous products water repellent and repellent to insects and fungi, and wherein the repellent properties thereof are obtained through treatment of the fiber, in dilute water suspension, with rosin size and sodium arsenate, the size and the arsenic thrown down on the fiber by the addition of alum. 115
28. The method of rendering vegetative fiber products water repellent, insect and fungi toxic, wherein the water repellent properties and toxicity are obtained through treatment of the fiber, in dilute water suspension, with rosin size 0.25 to 4% and sodium arsenate 0.005 to 0.40% (arsenic content), the arsenic and rosin thrown down on the fiber by the addition of alum to adjust the pH of 120

the suspension to between pH 4.0 and pH 7.5.

29. The method of rendering vegetative fiber products water repellent, insect and fungi toxic, wherein the water repellent properties and toxicity are obtained through treatment of the fiber, in dilute water suspension, with wax size 0.5 to 10% and sodium arsenate 0.005 to 0.40% (arsenic content), the arsenic and wax thrown down on the fiber by the addition of alum to adjust the pH of the suspension to between pH 4.0 and pH 7.5.

30. A felted fibrous product composed of vegetative fiber and having distributed throughout the body thereof the reaction product of rosin size, sodium arsenate and a coagulant and precipitant thereof.

In testimony whereof, we have signed our names to this specification as of the 23rd day of December, A. D. 1930.

20 TREADWAY B. MUNROE.  
ELBERT C. LATHROP.

25

30

35

40

45

50

55

60

65